

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## BINDER FOR THE MANUFACTURE OF REFRACtORY CONDUCTORS.

1,026,344.

Specification of Letters Patent. Patented May 14, 1912.

No Drawing.

Application filed August 7, 1907. Serial No. 387,549.

*To all whom it may concern:*

Be it known that I, WILLIAM D. COOLIDGE, a citizen of the United States, residing at Schenectady, county of Schenectady, State 5 of New York, have invented certain new and useful Improvements in Binders for the Manufacture of Refractory Conductors, of which the following is a specification.

This invention relates to the production of 10 refractory electrical conductors suitable for use in incandescent lamps, electrical furnaces, and other apparatus.

My invention comprises a process whereby refractory material, even though non-ductile, 15 may be shaped into wires, plates, rods, or other forms, and then consolidated into a coherent conductor capable of converting electrical energy into light at enormously high temperatures.

According to my invention, a refractory 20 element, alloy, compound or mixture is incorporated in a metallic binder, and the product so obtained is squirted or otherwise shaped into rods or filaments and then treated to drive out the easily vaporizable material of the binder and to consolidate and sinter together the refractory residue.

My process is applicable to a great variety 25 of refractory metals and materials, such, for instance, as tungsten, molybdenum, boron, zirconium, tantalum, titanium, graphite, or compounds of alloys of any of these, or of other materials of the same general refractory nature.

As a binding material I use an alloy 30 containing cadmium, lead and mercury. The alloy may have the following proportions, cadmium 42 parts, mercury 53 parts, lead 5 parts. This binder does not appear to 35 chemically combine with the refractory material with which it is impregnated, and consequently the process of manufacture is applicable to all the materials above mentioned and to many others.

In general, the binding material serves to 40 give the body ductility and strength, and in some cases to increase its electrical conductivity. It is retained in the mixture only until the body has been worked or formed 45 into the desired shape. It is then driven out by heat treatment and leaves behind a refractory coherent wire or rod suitable for use in lamps.

In order that my invention may be easily 50 practised, I have hereinafter described the

process as applied to the metal tungsten, but this specific application is to be regarded as only typical and as showing but one of numerous applications.

Tungsten suitable for use according to my 60 process may be made by reduction of tungsten trioxide with hydrogen according to the general process well known to chemists. This reaction should be carefully conducted so that the tungsten powder will be finely 65 divided and of a high degree of purity.

To compound the binder for use with tungsten or other refractory powder, I melt 70 together the cadmium and lead and then add the mercury. I find that the alloy thus produced is homogeneous, and when partially cooled is smooth and plastic and may be readily impregnated with the tungsten powder by simply rubbing the two together in a chemist's mortar. The powder goes in 75 very readily and the binder can be heated relatively hot without danger that the components will separate,—in other words that the alloy will break up into its component elements. Tungsten may be added to the 80 extent of 30 to 50 per cent. by weight of the final mixture. I call the product a mixture because I do not at present believe that the tungsten alloys or combines in any way with the material of the binder. The mixture is 85 ductile and pliable and can be readily rolled or worked by any of the well known metal working processes.

To obtain wires, plates, rods or other 90 forms suitable for the construction of lamp filaments or other apparatus, I squirt or extrude the plastic mixture above mentioned through a die, for example, a diamond die, at the temperature at which the mixture is soft and workable, say 100 to 150 degrees C. 95 The material comes out as a smooth homogeneous wire, not only ductile and pliable, but also so tough that it can be given a sharp twist and then be straightened out without danger of rupture. It may be squirted in 100 sizes varying from large rods or plates down to wires having a diameter of 1 mill or even less, and can be readily rolled or worked by any of the well known metal working processes. The ductile wire is next cut to length 105 and bent into loops having the shape of lamp filaments. A bundle of these loops is placed on a piece of wire gauze mounted in a glass tube. The tube is then evacuated and heated by a Bunsen burner to drive 110

from the wires the easily vaporizable components. This baking operation is continued until most of the mercury and some of the cadmium are driven from the filaments.

5 Enough of the binder stays behind to hold the tungsten together and render the filaments strong enough for subsequent handling.

The baked filament loops above described 10 are next suspended in treating bottles and heated with current to drive out the remainder of the binder. Each loop can be suspended in a treating bottle between metal clamps. The treating bottle should be 15 evacuated with a good mechanical pump and should be maintained dry by the use of an absorbing agent, such as phosphorous pentoxide. I prefer to have this drying agent in close proximity to the filament, as in a 20 small dish placed immediately below the filament during treatment.

The treatment of the filament loop is carried out by passing a low current through the loop until the binder is driven out and 25 then a higher current for fifteen to thirty seconds or even for a minute. The high current sinters the residue and shrinks the loop into a compact homogeneous wire having a bright metallic surface. The sintered loop 30 is strong enough for commercial use in incandescent lamps and can be operated in lamps at a very high efficiency.

As a modification of the processes above described I may reduce the lead content to 35  $2\frac{1}{2}$  parts and add to the metallic binder  $2\frac{1}{2}$  parts bismuth. This bismuth comes out of the filamentary conductors during the heat treatment in much the same way that the cadmium and other components come out. 40 It probably comes out later, however, and therefore is effective in strengthening the

filaments during that interval of time when they are free from cadmium but not yet sintered and shrunk. Such a binding material—that is one containing cadmium, 45 lead, bismuth and mercury—comes within the terms of the annexed claims which specify that the binder is an alloy containing cadmium, lead, and mercury or is an amalgam containing cadmium and lead. 50

What I claim as new and desire to secure by Letters Patent of the United States, is:—

1. A composition of matter consisting of refractory metal powder bound together by an amalgam containing cadmium and lead. 55

2. A composition of matter consisting of refractory metal powder bound together by an alloy containing cadmium, lead and mercury. 60

3. A composition of matter consisting of powdered tungsten bound together by an amalgam containing cadmium and lead.

4. A composition of matter comprising powdered tungsten bound together by an alloy containing cadmium, lead and mercury. 65

5. A conductive pliant wire consisting of refractory metal powder bound together by an amalgam containing cadmium and lead adapted to be converted into a refractory 70 incandescent body by suitable heat treatment.

6. A conductive pliant wire consisting of powdered tungsten bound together by an amalgam containing cadmium and lead. 75

In witness whereof, I have hereunto set my hand this 2nd day of August, 1907.

WILLIAM D. COOLIDGE.

Witnesses:

BENJAMIN B. HULL,  
HELEN ORFORD.